

# UNITED STATES PATENT OFFICE.

EWALD TESSEN, OF ROSTOCK, GERMANY.

## COMPOSITION FOR REMOVING PAINT.

SPECIFICATION forming part of Letters Patent No. 521,834, dated June 26, 1894.

Application filed September 29, 1893. Serial No. 486,793. (No specimens.)

*To all whom it may concern:*

Be it known that I, EWALD TESSEN, a subject of the Grand Duke of Mecklenburg-Schwerin, residing at Rostock, in the Grand Duchy of Mecklenburg-Schwerin, German Empire, have invented a new and useful composition of matter to be used for the destruction or removal of paints or old dried layers of color from wood, stone, metal, and other materials, of which the following is a specification.

Before entering into the details of the composition, it may be said that hitherto a caustic lye or the flame of a benzene-lamp has been generally used for the above-named purpose. Much time is lost and the workman is highly molested by poisonous vapors when the paint is removed by a flame, and much the same is the case, when a caustic lye, as for instance spirit of sal ammoniac is employed. Moreover, these lyes, being liquid, run down on vertical surfaces, and it is, consequently, necessary to apply them several times, as by a single application only a thin layer, insufficient for a complete destruction, remains on the paint. The greatest drawback, however, is occasioned by the penetration of the lye into the wood, so that, when painting afterward with fresh oil-color, the oil becomes saponified, and the color does not dry at all. Nevertheless, caustic lye is still the best means known for quickly dissolving the said old paints, and it appears therefore desirable to bring the liquid lye into an unguentary state, so that it cannot run down, but remains sticking to the paint in a layer of the required thickness. Now, when using for the inspissation the substances chosen hitherto for such purpose, as for instance flour, dextrine, and the like, the disadvantage arises, that the gluten contained in those means, combines with the caustic alkali, so that, as a matter of course, the caustic alkali is hindered from penetrating into the paint, and, consequently, from destroying the same.

My invention, now, consists, first, in inspissating the caustic lye by means of carageen-slime, which, containing no gluten, does

not combine in a chemical sense with the lye, but causes the latter to acquire an unguentary consistency. It has been found, secondly, that the inspissated lye is prevented from penetrating into the wood, after the paint has been dissolved, by an addition of powdered chalk, and, thirdly, the compound is kept moist and pliant, and prevented from drying from the action of the air by an addition of oil-lime-soap. It is, finally, appropriate, to saturate the carageen-slime with borax so as to prevent it thereby from becoming putrid.

For manufacturing my new compound I boil two and one-half kilos of carageen with sixty kilos of water for two hours, and I mix the fifty kilos of slime obtained thereby with one-half kilo of borax, which soon dissolves. This mass is then mixed with twenty-five kilos of oil-lime-soap, and there are added to it, after cooling, one hundred and twenty-five kilos of a caustic lye of 40° Baumé. The compound is finished by the addition of one hundred kilos of powdered chalk, which may have been previously colored by two and one-half kilos of ultramarine-green.

Even a very old and very hard paint may be completely destroyed and removed by covering it once with a sufficient layer of the above described compound, and letting the same act for about six hours.

What I claim, and desire to secure by Letters Patent, is—

As a means for destroying, and removing paints or old and dry layers of color, a composition of matter consisting of eight per cent. oil-lime-soap, sixteen per cent. carageen-slime, thirty-four per cent. chalk and forty-two per cent. caustic lye, substantially as described.

In testimony whereof I have signed this specification in the presence of two subscribing witnesses.

EWALD TESSEN.

Witnesses:

R. HERPICH,  
H. GENEHR.